

1

2,856,363

## STABLE ANTI-RUST LUBRICATING OIL

Elmer W. Brennan, Dundee, Ill., assignor to The Pure Oil Company, Chicago, Ill., a corporation of Ohio

No Drawing. Application December 1, 1955  
Serial No. 550,504

9 Claims. (Cl. 252—33.6)

This invention relates to a stable anti-rust lubricating oil composition containing certain epoxyalkaneamine reaction products which is characterized by its ability to pass the rust test designated as ASTM D665-50T and also by its good separation characteristics in the demulsibility test designated as ASTM D157-51T, the results being expressed as ASTM Steam Emulsion Number (S. E. No. ). These tests are well known and widely used and will hereinafter be referred to as the rust test and steam emulsion number.

The protection of metallic equipment from rusting has been a problem of long standing. A particularly acute problem has been the prevention of the rusting of ferrous parts operating in an environment wherein water from various sources mixes with the lubricant as in steam-turbine oils. Passage of the rust test, as above designated, is one of the critical factors in the formulation of satisfactory steam-turbine oils. For this purpose, there are available various rust inhibitors which have different degrees of effectiveness.

It has been found that even among inhibitors of the same generic class there is a wide variation in ability to carry a formulation through the rust test. In particular, it has been found that only certain amino-alcohol compounds are effective for this purpose.

Previous independent experiments on a number of rust inhibitors and related polymers had indicated that if the addend failed to pass the ASTM-D665 Rust Test, method A using distilled water, it also failed the method B test using synthetic sea water. Some of the addends tested included the co-polymers of styrene oxide and such materials as propylene sulfide, 2-mercaptopropyl dibutylamine and 2-hydroxypropyl dibutyl amine. These materials failed the ASTM-D665 Rust Test (method A) when used in amounts ranging from 0.05 to 2.0 weight percent. It was also found that other amino compounds such as tetramethyldiaminodiphenylmethane, dibutyl amine, triamylamine, aniline, methylaniline, dimethyl-aniline, tribenzylamine, and triethanolamine, when tested in amounts ranging from 0.1 to 0.5 weight percent in a base oil, were ineffective in passing the rust test.

In addition, it has been discovered that certain inhibitors, though very effective in their ability to prevent rusting, cannot be used because of emulsification and/or decreased stability of the composition in the presence of steam. For example, compounds such as tris (hydroxymethyl) aminomethane, although an effective rust inhibitor, was also an excellent emulsifying agent and could not be used because of emulsibility troubles. My invention resides in the discovery that amino-alcohols not only are excellent rust inhibitors but also do not adversely affect the demulsibility or steam emulsion number of the composition as do other related members of the class.

Accordingly, it is a primary object of my invention to provide a composition for inhibiting the rusting of metallic surfaces.

Another object of the invention is to provide a rust-inhibiting composition of matter exhibiting resistance to emulsion in the presence of water.

Still another object is to provide a stable anti-rust lubricating oil composition containing certain amino-alcohols.

2

A further object of the invention is to provide a stable anti-rust lubricating oil composition containing certain amino-alcohols prepared by the condensation or reaction of certain alkanolamines with epoxylkanes.

5 A further object is to provide a steam-turbine oil composition, containing among other ingredients a small amount of at least one of the above-defined amino-alcohol compounds, which is characterized by its ability to pass the rust test and which exhibits a satisfactory steam emulsion number as herein defined.

These and other objects of my invention will be described or become apparent as the description thereof proceeds.

Broadly, the inhibitors of the present invention comprise the reaction products of epoxylkanes and mono-alkanolamines or dialkanolamines. Although epoxylkanes may be condensed with alkyl amines or with triethanolamines, such reaction products are not suitable rust inhibitors. The general reaction forming the amino-alcohol inhibitors of this invention may be represented as follows:



25 Epoxyalkane Alkanolamine Amino-alcohol  
wherein R is an alkyl group having from 2 to 12 carbon atoms, R' may be hydrogen or an alkyl group of 2 to 12 carbon atoms, R'' is a hydrocarbon chain having from 2 to 5 carbon atoms and Y may comprise hydrogen or another R''—OH grouping. R'' may carry methyl substituents to increase the oil solubility. Specific examples are the condensation product of 1,2-epoxydodecane and 30 monoethanolamine and the condensation product of 1,2-epoxydodecane and diethanolamine. These compounds have the formulae



40 and



and are designated for purposes of the claimed invention as 2-hydroxy dodecane-1-monoethanolamine and 2-hydroxy dodecane-1-diethanolamine.

45 The epoxylkanes used in preparing the aforementioned amino-alcohols are selected from a wide group of straight chain epoxy compounds known and used in organic synthesis. The epoxylkanes are prepared by reaction of an unsaturated aliphatic hydrocarbon, having its double bond either between the terminal carbon atoms of the chain or located between carbon atoms which are located within the middle portion of the carbon chain, with hypochlorous acid, by oxidation, or by epoxidation. In the reaction with hypochlorous acid the chlorohydrin derivative is formed in the first step, and is transformed to the epoxide by dehydrochlorination with an alkali, such as sodium hydroxide. In each reaction the result is the placement of a single oxygen atom across the double carbon atom bond.

55 The epoxylkanes include the epoxides of the following unsaturated aliphatic hydrocarbons: butene-1, pentene-1, hexene-1, heptene-1, octene-1, nonene-1, decene-1, undecene-1 and dodecene-1 as the aliphatic olefins, wherein a single oxygen atom is linked across adjacent carbon atoms at the double bond. The various structural isomers of these, wherein the



70 linkage is not at a terminal carbon atom, or the chain is branched, include the epoxides of butene-2, isobutylene,

pentene-2, 2-methyl-butene-1, 2-methyl-butene-2, 3-methyl-butene-1, 3-methyl-pentene-2, tetramethylethylene, tertiary-butylethylene, the heptylenes and the octylenes.

The alkanolamines which are reacted with the aforementioned epoxides to form my amino-alcohol inhibitors include only the mono-alkanolamines and the dialkanolamines. Monoethanolamine, diethanolamine, propanolamine, monoisopropanolamine, 2-amino-1-propanol, 3-amino-1-butanol, 2-amino-2-methyl-1-propanol, dipropylamine, and dibutanolamine are included in this group of alkanolamines which may have from 2 to 11 carbon atoms in the molecule. Preferably, the hydroxyl group and the amino group are at opposite ends of the molecule.

The reaction by which the alkanolamine and the epoxyalkanes are condensed is very simply carried out, since no catalysts or solvents are required. According to Huscher and Long in United States Patent 2,602,819, in using the lower molecular weight epoxyalkanes it is only necessary to place the alkanolamine, in anhydrous condition, into a reaction vessel fitted with cooling means and slowly add the epoxyalkane. The rate of addition of the epoxyalkane is used to control the reaction temperature. Since the epoxyalkane may be lost by evaporation it is advisable to conduct the reaction under reflux or in a closed vessel at a pressure at least equal to the autogenous pressure of the reaction mixture to prevent such loss. The pressures used do not generally exceed 2-3 atmospheres. The reaction proceeds rapidly and is completed within a few hours, at the most, after the addition of the epoxyalkane is finished. Evolution of heat ceases upon completion of the reaction. The reaction temperature, which may start at 0° C., should be controlled to avoid exceeding about 100° C. in order to prevent the formation of undesirable by-products. The reaction of 20 gram-mols of propylene oxide with 10 gram-mols of monoisopropanolamine takes place at room temperature in a closed vessel to form a predominance of tri-isopropanolamine.

Usually, the proportion of epoxyalkane to alkanolamine used will be no more than 2:1 when the reactant is monoalkanolamine and not more than 1:1 when the reactant is dialkanolamine. For the reaction of higher molecular weight epoxyalkanes having from 6 to 12 carbon atoms, the reaction may be carried out by the method described in United States Patent 2,373,199 by subjecting a molecular excess of a mono-alkanolamine to reaction with an epoxyalkane at higher temperatures, between 120 to 275° C., under pressures up to 1000 pounds per square inch. Reaction of 6 gram-mols of monoethanolamine with 1 gram-mol of ethylene oxide at 150° C. and 485 pounds per square inch pressure, using the U. S. 2,373,199 method, results in a 78% conversion to monoethyl amino ethanol and a 19.6% conversion to monoethyl diethylolamine.

The epoxyalkane-amine reaction products of this invention are not to be confused with the high molecular weight polymeric materials formed in accordance with such prior art processes as disclosed in United States Patents 2,522,155 and 2,498,195 by Ballard, Morris and Van Winkel, or the products of the process of United States Patent 1,920,578 by Schoeller and Wittwer. These condensation products have a plurality of -(O-R)- groups in the molecule and are of high molecular weight and polymeric in nature.

In order to demonstrate the invention, a number of steam-turbine oil compositions were prepared from a base oil composition which contained the following ingredients:

Table I

|                  | Wt. percent |
|------------------|-------------|
| Mineral oil      | 99.518      |
| Paranox 441      | 0.35        |
| Age Rite Stalite | 0.12        |
| Butyl zimate     | 0.012       |

The mineral oil was composed of 27 wt. percent of Mid-Continent, solvent-refined neutral oil which had the following characteristics: viscosity at 100° F., 82.1 SUS; viscosity at 210° F., SUS 37.9; 103 V. I.; C. R., con. percent, 0.00; flash, COC, ° F., 390; fire, COC, ° F., 425; gravity, API, 35.5; pour, ASTM, ° F., 0.00; and 72.51 wt. percent of Mid-Continent, solvent-refined neutral oil which had the following characteristics: carbon residue (Conradson), 0.01%; flash, COC, 415° F.; fire, COC, 480° F.; API gravity, 31.3°; pour, 0° F.; viscosity at 100° F., SUS, 178; viscosity at 210° F., SUS, 46.2; and a V. I. of 100. This composite base oil had a carbon residue (Conradson) of 0.01%; flash, COC, 400° F.; fire, COC, 455° F.; API gravity, 32.8°; pour, 0° F.; viscosity at 100° F., 148 SUS; viscosity at 210° F., 43.1, SUS. Paranox 441 is a trade name for di-tertiary-butyl paracresol and is present in the composition for the purpose of inhibiting oxidation. Cresols generally, and especially this specific cresol, have no measurable ability to either inhibit or promote the formation of rust. Age Rite Stalite is a trade name for a mixture of octylated and styrenated diphenylamines. This aryl amine product is incorporated for the purpose of inhibiting oxidation, and has no particular anti-rust or rust-producing properties in itself. Butyl zimate is a zinc dibutylthiocarbamate and is used for the purpose of inhibiting oxidation. The combination of these three materials is a synergistic mixture for inhibiting oxidation.

The base composition may be varied somewhat from the weight percentages shown above. Up to 1.0 wt. percent of Paranox 441 may be used, depending upon the level of oxidation stability required or desired. The Age Rite Stalite may be present in amounts ranging up to 0.5 wt. percent, as long as a sufficient amount is present to adequately inhibit oxidation. Similarly, the butyl zimate may be used in amounts ranging up to 0.05 wt. percent.

Three different epoxyalkane-amine reaction products were used in these tests and the ability of equal amounts of these materials to inhibit rusting was evaluated. The results are shown in the following Table II:

| Composition, Percent Wt.              | Blend |       |       |
|---------------------------------------|-------|-------|-------|
|                                       | A     | B     | C     |
| Base Composition                      | 99.95 | 99.95 | 99.95 |
| 1,2-Epoxydodecane-dibutylamine        | .05   |       |       |
| 1,2-Epoxydodecane-monoethanolamine    |       | .05   |       |
| 1,2-Epoxydodecane-diethanolamine      |       |       | .05   |
| ASTM-D655-50T Rust Test:              |       |       |       |
| Method A (Distilled H <sub>2</sub> O) | Fail  | Pass  | Pass  |
| Method B (Syn. Sea H <sub>2</sub> O)  | Fail  | Pass  | Fail  |
| ASTM D157-51T (SE No.)                | 85    | 198   | 77    |

It is seen from the above experiments that the epoxyalkane-alkanolamine reaction products were effective rust inhibitors in comparison to the unsatisfactory epoxyalkane-alkylamine product, and that the epoxyalkane-mono-alkanolamine product was the more effective for both distilled and sea water at the concentration level shown. Both of the preferred compounds give a satisfactory Steam Emulsion No. for the oil. The blank oil had a Steam Emulsion Number of 40.

The condensation product of 1,2-epoxydodecane and monoethanolamine was prepared by reacting 14 parts of the epoxide with 18 parts of monoethanolamine by refluxing the materials for 4 hours. The dibutylamine and diethanolamine reaction products were similarly prepared. From this it is seen that the monoethanolamine reaction product is superior to the dibutylamine and diethanolamine reaction products in rust inhibiting properties. Effective concentrations of the alkene epoxide-monoalkanolamine reaction product may be between 0.01 and 0.5 weight percent, but in general, a concentration of about 0.05 weight percent is sufficient for all purposes. The 1,2-epoxydodecane-diethanolamine prod-

uct finds its usefulness in those applications where the coolant water that may contaminate the lubricant is land water. The 1,2 epoxidodecane-monoethanolamine product extends the usefulness to use aboard ship, for example, where sea water contamination presents a serious corrosion problem.

What is claimed is:

1. A lubricating oil composition characterized by its oxidation stability and its ability to pass the ASTM-D665 Rust Test, comprising a major amount of mineral lubricating oil, an oxidation inhibitor combination comprising about 0.35 weight percent of di-tertiary butyl para-cresol, about 0.12 weight percent of a mixture of octylated and styrenated diphenyl amines, about 0.012 weight percent of zinc dibutyl-dithiocarbamate, and about 0.01 to 0.5 weight percent of an amino-alcohol having the general formula:



wherein R is an alkyl group having from 2 to 12 carbon atoms, R' is selected from the group of hydrogen and an alkyl group of 2 to 12 carbon atoms, R'' is a hydrocarbon chain having 2 to 5 carbon atoms and Y is selected from the group of hydrogen and an R''—OH group.

2. A lubricating oil composition in accordance with claim 1 in which R is an alkyl group having 10 carbon atoms, R' is hydrogen, R'' is a hydrocarbon chain having 2 carbon atoms and Y is hydrogen.

3. A lubricating oil composition in accordance with claim 1 in which R is an alkyl group having 10 carbon atoms, R' is hydrogen, R'' is a hydrocarbon chain having 10 carbon atoms and Y is hydrogen.

4. A lubricating oil composition in accordance with claim 1 in which the amino-alcohol is 2-hydroxy dodecane-1-diethanolamine.

5. A lubricating oil composition in accordance with claim 1 in which the amino-alcohol is a 2-hydroxy dodecane-1-monoethanolamine.

6. A steam-turbine oil comprising about 25 volume percent of 85 viscosity neutral oil and 74.46 volume percent

of a 175 viscosity neutral oil, about 0.35 weight percent of di-tertiary butyl para-cresol, about 0.12 weight percent of a mixture of octylated and styrenated diphenyl amines, about 0.012 weight percent of zinc dibutyl-dithiocarbamate and about 0.05 weight percent of 2-hydroxy dodecane-1-diethanolamine, said composition being characterized by its ability to pass the ASTM-D665 Rust Test.

7. A steam-turbine oil comprising about 25 volume percent of 85 viscosity neutral oil and 74.46 volume percent of a 175 viscosity neutral oil, about 0.35 weight percent of di-tertiary-butyl para-cresol, about 0.12 weight percent of a mixture of octylated and styrenated diphenylamines, about 0.012 weight percent of zinc dibutyl-dithiocarbamate, and about 0.05 weight percent of 2-hydroxy dodecane-1-monoethanolamine, said composition being characterized by its ability to pass the ASTM-D665 rust test.

8. A lubricating oil composition characterized by its ability to pass the ASTM-D665 Rust Test, comprising a major portion of a mineral lubricating oil containing about 0.35 weight percent of di-tertiary-butyl para-cresol, about 0.12 weight percent of a mixture of octylated and styrenated diphenylamines, about 0.012 weight percent of zinc dibutyl-dithiocarbamate, and about 0.05 weight percent of 2-hydroxy dodecane-1-monoethanolamine.

9. A lubricating oil composition characterized by its ability to pass the ASTM-D665 Rust Test, comprising a major portion of a mineral lubricating oil containing about 0.35 weight percent of di-tertiary-butyl para-cresol, about 0.12 weight percent of a mixture of octylated and styrenated diphenylamines, about 0.012 weight percent of zinc dibutyl-dithiocarbamate, and about 0.05 weight percent of 2-hydroxy dodecane-1-diethanolamine.

35  
 References Cited in the file of this patent  
 UNITED STATES PATENTS  
 2,497,553 Long \_\_\_\_\_ Feb. 14, 1950  
 2,522,155 Ballard et al. \_\_\_\_\_ Sept. 12, 1950  
 2,602,819 Huscher et al. \_\_\_\_\_ July 8, 1952  
 2,605,224 Jahn \_\_\_\_\_ July 29, 1952  
 2,629,694 Woods et al. \_\_\_\_\_ Feb. 24, 1953